

1

2,899,262

## METHOD AND COMPOSITION FOR RENDERING POLYACRYLONITRILE READILY DYEABLE

George W. Stanton, Walnut Creek, Theodore B. Leffer-dink and Richard W. Meikle, Concord, and Mary J. Charlesworth, Walnut Creek, Calif., assignors to The Dow Chemical Company, Midland, Mich., a corporation of Delaware

No Drawing. Application April 6, 1953  
Serial No. 347,144

4 Claims. (Cl. 8—100)

This invention relates to a readily dyeable composition of polyacrylonitrile or of copolymers containing at least 85 percent by weight of acrylonitrile in the polymer molecule, to fibrous articles made from such compositions, and to a method of making such polymers readily dyeable. It relates as well to a method of dyeing such polymers.

It is known that polyacrylonitrile and copolymers containing 85 percent or more of acrylonitrile can be spun to form useful fibers. It is also known that, when spun from organic solvents, they can only be dyed with great difficulty unless the fibers have been stretched so little as to have a low tenacity or unless the polymeric structure includes reactive groups to bind a limited class of dyes. It has been proposed, also, to blend such dye assistants as polyvinylpyridine with polyacrylonitrile, and to dissolve and spin the mixture. Such additives make difficult control of the spinning procedure and of the fiber properties. The polymeric acrylonitrile can be dissolved in and spun from aqueous solutions of various highly hydrated metal salts. When such saline solutions are extruded through spinnerets into aqueous coagulants, such as water, dilute brines or dilute acids, there is formed a swollen aquagel structure from which strong, useful fibers can be formed by a series of stretching, washing and drying operations. When such fibers are dried, they are as hydrophobic as the ones obtained from organic solutions of the same polymers, and present the same difficulties when it is desired to dye them. It has been proposed, however, to dye the fibers during the course of their production, using an aqueous dye bath, and applying the dye to the fiber while the latter is in the swollen aquagel condition, before it has been subjected to irreversible drying. The so-outlined procedure has made possible better dyeing of acrylonitrile polymer fibers than has been obtained with fibers of the same polymers spun from organic solvents, but it has a serious disadvantage. The textile industry prefers to purchase fibers in an undyed condition so as to have complete freedom of choice as to color and shade of the manufactured goods. If fibers can only be obtained in a ready-dyed state or in an undyeable state, the textile industry is understandably reluctant to use such fibers. It is also reluctant to acquire and use a swollen aquagel, since standard yarn and fabric making equipment is designed for more rugged raw materials, and the aquagel must be dried before the fiber has its desirable properties.

The foregoing statement of the problem has referred to fibers and products made from them, and the invention will be illustrated with respect to fibers. The problem is more general, however, and applies to the defined compositions in the forms of films or sheets, tubes, rods and molded articles as well as fibers and other filaments.

It is among the objects of this invention to facilitate the dyeing of structures such as fibers and films of poly-

2

meric bodies containing at least 85 percent of acrylonitrile in the polymer molecule. A related object is to provide a method whereby such structures, made by coagulation of aqueous saline solutions of the polymer, may be treated so as to be dyeable after they have been dried. A particular object is to provide such polymeric articles and compositions which can be dyed readily with any common dye.

The invention is based on the discovery that readily dyeable oriented products may be made from the defined high acrylonitrile polymers by incorporating in the spun article during the course of its manufacture and before it is dried and reduced to its final dimensions, a particular type of dye assistant to be defined hereinafter, and subsequently freeing the article from the saline medium while leaving the assistant in the dried product. By the reference to adding the assistant to the product "during the course of its manufacture" is meant introduction of the assistant into the coagulated and still swollen spun product, before or after partial orientation. The invention is applicable to products made by wet-spinning of aqueous saline solutions of the polymer.

According to the present invention, a polymer containing at least 85 percent acrylonitrile in the polymer molecule is spun from an aqueous saline solution thereof into an aqueous coagulant, and the coagulated product is stretched to effect orientation and is washed in any conventional manner to extract saline constituents. The amount of stretching imparted should be sufficient to give a product having a yield point, when dried, of at least 0.8 gram per denier, as less fully oriented products, those with yield points near 0.6 gram per denier or less, may be dyed relatively easily. Either before or after the initial coagulation, and while the product is still an aquagel, i.e., before it has been dried irreversibly, and preferably after most of the inorganic salt has been removed, a water-soluble dye assistant, of a type to be defined hereinafter, is applied to and absorbed by the aquagel product in amount to represent at least 1.0 percent of the dry weight of the polymeric product. Thereafter, the product is dried, while still retaining the dye assistant. The product may then be packaged, stored, and subjected to fabrication steps, such as carding, twisting, spooling and knitting or weaving, if desired, before being dyed. Any common type of dye may be used, and the dyeing procedure may be one which needs, at most, only slight modification from that recommended for use with that dye when applied to the fibers (wool, cotton, silk, viscose or acetate rayon, or nylon) for which the dye is primarily intended. Many of the useful procedures are outlined hereinafter.

The dye assistants of the present invention are significantly water-soluble salts of a member of the group: (a) polyalkylene amines, (b) fatty acid amides of such amines, (c) N-alkyl and carboxyalkyl derivatives of such amines, (d) N-alkyl and carboxyalkyl derivatives of the fatty acid amides of such amines, and (e) condensation products of aldehydes with such amines, in all of which the polyalkylene amine has a molecular weight of at least 200. The polyalkylene amines all contain secondary amine groups, and, with reference to such groups, they may be called polyalkylene imines. The salts are hydrohalides, alkyl acid sulfates or any other significantly water-soluble salts of the polyalkylene amines. The alkylene groups in such amines may be the ethylene, propylene or butylene radicals. When the polyalkylene amines have molecular weights below 200, their salts do not have the permanence required of a dye assistant in the invention, and when their molecular weights are over about 15,000, their salts may have too little solubility in water to be as useful as desired.

Examples of the dye assistants of the present invention, all of which are effective in the process, are:

- (1) Polyethylene amine hydrochloride.
- (2) Polypropylene amine hydrobromide.
- (3) Polyethylene amine bis lauryl amide hydrochloride.
- (4) Polyethylene amine tetrastearamide hydrochloride.
- (5) Condensation product of (1) with alkyl halides or sodium chloroacetate.
- (6) Condensation product of (3) with alkyl halides or sodium chloroacetate.
- (7) Condensation product of (1) with formaldehyde.

All of these compounds are salts of polyalkylene amines and will be referred to as such herein.

In the method of the invention as applied to salt spun fibers, the time actually required for the water-swollen fiber to absorb the dye assistant is very brief, and varies with the degree of swelling of the fiber, the concentration of the liquid from which the assistant is applied, and the temperature of application. In some instances, enough of the assistant has been absorbed by the swollen fibers in 2 seconds. No adverse effect is found when the fibrous aquagel is soaked in the assistant for several days. The assistant may be used at full strength or in aqueous solutions which may be of any desired or convenient concentration. Thus, solutions containing as little as 0.1 percent by weight of the assistant have been used successfully. The assistant or its solution should be at a pH from 1 to 7, and should preferably be at a pH below 6, when applied to fibers in the swollen aquagel condition. The time and temperature of treatment, and concentration of the treating liquid should be so correlated as to cause the fibers to absorb at least 1.0 percent of their dry weight of the assistant. Amounts of 2 to 15 percent are preferred, but amounts as high as 40 percent are unobjectionable, though such large amounts are considered uneconomical. The temperature of treatment may be any temperature at which the aquagel fibers exist and at which the assistant or its solution is liquid. It is convenient to effect the treatment at room temperature or at temperatures up to about 100° C., but temperatures of 10° C. or lower may be used if desired.

The salts of polyalkylene amines are applied to the spun polyacrylonitrile, while the latter is in the aquagel condition, from aqueous solutions of at least 0.1 percent concentration (preferably 0.3 to 1 percent), under conditions of time and temperature such that the swollen fibers take up at least 1 percent of the assistant, based on the dry weight of the polymer in the fiber.

The importance of absorbing the dye assistant in the undried and still swollen form of the fiber is illustrated in the following table. One sample of the fiber was treated as an aquagel with the identified dye assistant until it had absorbed 1.0 percent of the fiber dry weight of that agent. Another sample was dried and then soaked in the same agent until it would remove 5.0 percent of its weight of the agent from the bath. Both fibers were boiled in identical baths of "Xylene Milling Blue FF" containing 2 percent of the dye, 10 percent of sodium sulfate, and 2 percent of acetic acid, all percentages being based on the dry weight of the fibers.

| Dye Assistant                                      | Application and conc. on Fiber    | Percent Exhaustion of Dye Bath | Remarks            |
|----------------------------------------------------|-----------------------------------|--------------------------------|--------------------|
| Polyethylene amine bis lauryl amide hydrochloride. | 1.0 percent applied to aquagel.   | about 60..                     | Excellent dyeing.  |
| Do-----                                            | 5.0 percent applied to dry fiber. | about 15..                     | Negligible dyeing. |

The assistants have a greater affinity for the swollen aquagel than for their own aqueous solutions. Thus, when the aquagel is soaked in solutions of the assistants until equilibrium is reached, a 0.1 percent solution may leave about 1.5 percent of the assistant in the fiber and a 1.0 percent solution may leave as much as 10 percent of the assistant in the fiber, at room temperature. At a given concentration of the assistant in water, the amount which can be absorbed by the swollen fibers remains about constant for temperatures from 15° to 45° C., but a further increase in temperature to about 85° C. results in nearly twice as much of the assistant becoming absorbed in the fiber. Satisfactory dyeing is obtained whenever the fiber has been treated to carry 1.0 percent or more of its dry weight of the assistant, and the heaviest dyeing is found with fibers which carry over 1.5 percent of the assistant. There is no advantage to be gained through using over 40 percent of the assistant on the fibers.

The dye assistants of the present invention, when absorbed as described on the aquagel fibers, have made the subsequently dried fibers dyeable, using common classes of dyes including direct cotton and azoic dyes; vats; soluble vats; acid, acid-mordant and basic dyes; and acetate dyes. The following is a list of representative dyes which have been applied successfully by the present method. So far as possible, the Colour Index number of the dye is given, or the number of the recognized foreign prototype (marked "PR") of the American dye employed, as listed in various editions of the "Yearbook of the American Association of Textile Chemists and Colorists." In those cases in which neither a "C.I." nor a "PR" number is reported, the dye definitely belongs to the class with which it is reported.

|                                                 | C.I.   |
|-------------------------------------------------|--------|
| (a) Direct cotton dyes:                         |        |
| Chlorantine Fast Brown CLL                      |        |
| Chlorantine Fast Green 5BLL                     | PR 470 |
| Chlorantine Fast Red 7B                         | 278    |
| Pontamine Green GX Conc. 125%                   | 594    |
| Calcomine Black EXN Conc                        | 581    |
| Niagara Blue NR                                 |        |
| Erie Fast Scarlet 4BA                           | 326    |
| (b) Acid dyes:                                  |        |
| Anthraquinone Green GN                          | 1078   |
| Anthraquinone Blue AB                           | 1075   |
| Sulfonine Brown 2R                              |        |
| Sulfonine Yellow 2G                             | 642    |
| Neutracyl Brown RD                              |        |
| Xylene Milling Black 2B                         | 304    |
| Xylene Milling Blue FF                          |        |
| Xylene Fast Rubine 3GP PAT                      | PR 412 |
| Calcocid Navy Blue R Conc                       | 289    |
| Calcocid Navy Fast Blue BL                      | 833    |
| Calcocid Milling Red 3R                         | 275    |
| Alizarine Levelling Blue 2R                     |        |
| Amacid Azo Yellow G Extra                       | 146    |
| (c) Mordant-acid dyes:                          |        |
| Alizarine Light Green GS                        | 1078   |
| Brilliant Alizarine Sky Blue BS PAT             | 1088   |
| (d) Basic dyes:                                 |        |
| Brilliant Green Crystals                        | 662    |
| Du Pont Methylene Blue ZX                       | 922    |
| Rhodamine B Extra S                             | 749    |
| (e) Vat dyes:                                   |        |
| Midland Vat Blue R Powder                       | 1183   |
| Sulfanthenre Brown G Paste                      | PR 121 |
| Sulfanthenre Black PG Dbl. Paste                |        |
| Sulfanthenre Blue 2B Dbl. Paste                 | 1184   |
| Sulfanthenre Red 3B Paste                       | 1212   |
| (f) Soluble vat dyes: Indigosol Green IB Powder |        |
| (g) Acetate dyes:                               |        |
| Celliton Fast Brown 3RA Extra CF                | PR 230 |
| Celliton Fast Rubine BA CF                      | PR 238 |

|                                                            |       |
|------------------------------------------------------------|-------|
| Artisil Direct Black BKZ                                   |       |
| Artisil Direct Navy BR                                     |       |
| Artisil Direct Red 3BP                                     | PR 61 |
| Celanthrene Pure Blue BRS 400%                             |       |
| Celanthrene Red 3BN Conc.                                  | PR 61 |
| Acetamine Orange 3R Conc.                                  |       |
| Acetamine Yellow N                                         |       |
| (h) Azoic dyes: $\beta$ -Naphthol-2-chloro-4-nitro-aniline |       |

The following typical procedures have been used successfully in dyeing the treated fibers of this invention.

(1) Direct cotton dyes:

Bath to fiber ratio, 40-80:1  
Dye to fiber ratio, 0.02-0.05:1  
Sodium sulfate to fiber, .10-.15:1  
Bath temperature, 100° C.  
Time, 1-1.5 hours  
Rinse in distilled water and dry

(2) Acid dyes:

Bath to fiber ratio, 30-40:1  
Dye to fiber ratio, .02-.05:1  
Sodium sulfate, .10-20:1  
Acetic acid, .02-.05:1 (for milling dyes), or  
Sulfuric acid, .02-.05:1 (for levelling dyes)  
Bath temperatures, 100° C. (boil)  
Rinse and dry

(3) Acetate dyes:

Bath to fiber ratio, 30-40:1  
Dye to fiber ratio, 0.02-.05:1  
Nonionic wetting agent, 0.1% or less.  
Bath temperature, 100° C. (boil) about 1 hour.  
Rinse and dry

(4) Soluble vat (procedure for Indigosol Green IB):

Dissolve dyestuff in hot water containing 1 gram per liter of sodium carbonate. Add 1 percent sodium hydrosulfite and 20 to 40 percent sodium sulfate. Enter goods at 40° C., heat within 30 minutes to 90° C. Hold near 90° C. for 1 hour. Rinse.

Prepare developing bath of 1 to 2 percent each of ammonium thiocyanate and potassium dichromate. Treat goods in this bath 30 minutes at 30° C. Add 10 grams sulfuric acid per liter, heat within 30 minutes to 85° C. and hold at 85°-90° C. for 30 minutes. Rinse thoroughly, neutralize with dilute (2 grams per liter) sodium carbonate, rinse again and scour.

(5) Vat: Procedure varies with the dye employed. For a satisfactory procedure when using sulfanthrene vat dyes, see Example 6, below.

The following specific examples illustrate the practice of the invention:

*Example 1*

A length (9 gms.) of water-swollen, unstretched tow, formed by extrusion of an aqueous saline solution of polyacrylonitrile through a 10 mil, 300 hole metal spinneret into an aqueous coagulating bath, was washed thoroughly to remove salt. It was then allowed to stand in 500 mls. of a 0.4% solution of polyethylene amine tetraesteramide hydrochloride (M.W. of amine over 1800) held at pH 3 with HCl at 25° C. until the fibers had absorbed at least 1 percent of the assistant. The tow was removed from the impregnating solution, stretched to 10 times its original length in moist steam, blown in a stream of air, and then dried for 8 minutes at 150° C. under little or no tension. The fibers had a tenacity of over 2 grams per denier.

The dried, impregnated tow was immersed in an aqueous dye bath containing 4.0% Pontamine Green GX Conc. 125% (C.I. 594) and 15.0% sodium sulfate, both percentages being based on the weight of the fiber. The dye bath to fiber ratio was 40 to 1. The dye bath was

held at 100° C. for 1.5 hours at which time the dye bath was completely exhausted. The dyed tow was removed, rinsed thoroughly in distilled water, and dried at 100° C. for 0.5 hour. The tow was dyed a deep, level green.

*Example 2*

A polyacrylonitrile tow was spun and washed as in Example 1. The water-swollen tow was stretched to 6 times its length while immersed for 4.5 seconds in an 10 0.8% aqueous solution of polyethylene amine tetraesteramide hydrochloride (M.W. of amine 1800) at 95° C. and held at pH 3 with HCl. The impregnated tow was stretched to 14.4 times its original length, in wet steam, and was dried on steam rolls, blown in an air 15 stream, and dried relaxed for 8 minutes at 150° C. This process was carried out continuously. The tow contained 3.0% of the additive. The tow was then dyed by the procedure of Example 1. After drying, the tow was dyed a deep, level green and contained 1.5% by weight of 20 dye. The tow dyed in Examples 1 and 2 had a light and crock fastness equal to cotton when dyed with the same dye and using the same procedure.

*Example 3*

25 A polyacrylonitrile tow was spun and washed as in Example 1. This tow was then stretched, impregnated with 3.6% octyl polyethylene amine hydrochloride (M.W. of amine about 650), and dried by the procedure of Example 2. The dried impregnated tow was immersed in 30 an aqueous dye bath containing 2.0% Xylene Milling Blue FF, 10% sodium sulfate, and 3-5% of acetic acid, all percentages being based on the weight of the fibers. The dye bath to fiber ratio was 40-1. The dye bath was held at 100° C. for one hour after which the tow 35 was thoroughly rinsed, and dried at 150° C. for 10 minutes. The tow was scoured with a 0.5% solution of a nonionic detergent at 60° C. for 15 minutes. The tow was dyed a level blue.

*Example 4*

40 A polyacrylonitrile tow was spun and washed as in Example 1. This tow was then stretched, impregnated with the hydrochloride of the condensation product of polyethylene amine (M.W. 5000) and sodium chloroacetate, and dried by the procedure of Example 2. The 45 dried impregnated tow was immersed in an aqueous dye bath containing 2% Acetamine Yellow CG and 0.1% of a nonionic wetting agent, both percentages being based on the weight of the fibers. The dye bath to fiber ratio was 30-1. The dye bath was held at 100° C. for 1.5 hours, after which the tow was thoroughly rinsed and 50 scoured with a 0.5% solution of a nonionic detergent at 60° C. for 15 minutes. A level yellow dyeing was obtained.

*Example 5*

55 A polyacrylonitrile tow was spun and washed as in Example 1. This tow was then stretched, impregnated with the hydrochloride of the bis lauryl amide of polyethylene amine (M.W. of amine over 600), and dried by 60 the procedure of Example 2. The dye bath was prepared by dissolving 2% Indigosol Green IB in hot water containing 1 gram per liter  $\text{Na}_2\text{CO}_3$ . One percent sodium hydrosulfite and twenty percent sodium sulfate were added. The tow was entered at 40° C. and heated with 65 in  $\frac{1}{2}$  hour to 90° C., then treated for 1 hour at 90-95° C. and finally rinsed. The dye bath to fiber ratio was 20-1. The developing bath was prepared with 1% ammonium thiocyanate and 1% potassium dichromate dissolved in water and the tow was treated in this bath for 70  $\frac{1}{2}$  hour at 30° C. Ten grams of concentrated sulfuric acid per liter of bath was then added and the bath was heated within  $\frac{1}{2}$  hour to 85° C. The bath was then held for  $\frac{1}{2}$  hour at 85-90° C. The tow was then rinsed thoroughly, neutralized with  $\text{Na}_2\text{CO}_3$  and rinsed again. The tow was dyed a level green.

*Example 6*

A polyacrylonitrile tow was spun and washed as in Example 1. This tow was then stretched, impregnated with the hydrochloride of the reaction product of polyethylene amine (M.W. 1800) with 4 moles of formaldehyde, and dried by the procedure of Example 2. A dye bath was then prepared with 4% Sulfanethrene Red 3B paste, 10% sodium hydroxide, and 10% sodium hydrosulfite. The tow was entered into the dye bath at a ratio of 20-1. The bath was held at 100° C. for 1/2 hour after which the tow was entered into an oxidizing bath of 4% hydrogen peroxide. The tow was then rinsed with cold water, neutralized with Na<sub>2</sub>CO<sub>3</sub>, and rinsed again and had a uniform red color.

*Example 7*

A polyacrylonitrile tow was spun and washed as in Example 1. This tow was then stretched, impregnated with the same assistant as in Example 6, and dried by the procedure of Example 2. The dried impregnated tow was immersed in an aqueous dye bath containing 3.0% Pontamine Green GX Conc. 125% and 15% sodium sulfate. The dye bath to fiber ratio was 40-1. The dye bath was held at 100° C. for 1.5 hours, following which the tow was rinsed and dried for 10 minutes at 150° C. The tow was then immersed in a bath containing 2% potassium dichromate and 2% acetic acid. The bath to fiber ratio was 40-1. This bath was held at 60° C. for 1/2 hour following which the tow was rinsed and dried. The product was dyed a level green.

*Example 8*

A polyacrylonitrile tow was spun and washed as in Example 1. This tow was then stretched, impregnated with the same assistant as in Example 5, and dried by the procedure of Example 2. The dried impregnated tow was padded with Naphtholate AS after which the tow was entered into a bath containing diazotized 2-chloro-4-nitroaniline. The bath was held at 95-100° C. for 1/2 hour, following which the tow was blotted dry. The tow was then entered into a developing bath consisting of 1.5% acetic acid, 0.75% formic acid, and 3.3% sodium

sulfate. The bath-fiber ratio was 15:1. This bath was held at 95-100° C. for 1/2 hour after which the tow was rinsed and dried. The tow was dyed a deep level red.

We claim:

- 5 1. In a process in which a polymer containing at least 85 percent of acrylonitrile in the polymer molecule is spun from an aqueous saline solution thereof into an aqueous coagulant, the spun product is stretched to an extent sufficient to yield a dried product having a yield point of at least 0.8 gram per denier, and the stretched product is substantially freed from saline constituents and dried to destroy the aquagel condition, the improvement which consists in: applying to the product while still in the aquagel condition at least 1.0 percent of its dry weight of a water-soluble salt of an N-carboxyalkyl derivative of a polyethylene amine having a molecular weight of at least 200, drying the so-treated product irreversibly, and thereafter dyeing the product.
- 10 2. The method claimed in claim 1, wherein the polymer subjected to spinning is polyacrylonitrile.
- 15 3. The method claimed in claim 1, wherein the dye assistant is the hydrochloride of a carboxymethylated polyethylene amine.
- 20 4. A dyeable fiber of a linear polymer containing at least 85 percent acrylonitrile in the polymer molecule, carrying uniformly distributed therethrough at least 1.0 percent of its dry weight of a water-soluble salt of an N-carboxyalkyl derivative of a polyethylene amine having a molecular weight of at least 200.
- 25

## References Cited in the file of this patent

## UNITED STATES PATENTS

|           |           |               |
|-----------|-----------|---------------|
| 1,985,248 | Ellis     | Dec. 25, 1934 |
| 2,135,633 | Bienert   | Nov. 8, 1938  |
| 2,347,508 | Rugeley   | Apr. 25, 1944 |
| 2,376,891 | Alles     | May 29, 1945  |
| 2,558,735 | Cresswell | July 3, 1951  |

## FOREIGN PATENTS

|         |               |               |
|---------|---------------|---------------|
| 361,362 | Great Britain | Nov. 16, 1931 |
| 613,817 | Great Britain | Dec. 3, 1948  |
| 613,818 | Great Britain | Dec. 3, 1948  |